# EUROPEAN PATENT SPECIFICATION

(11) **EP 0 714 773 B1**
(45) Date of publication and mention of the grant of the patent: **13.10.1999**
(21) Application number: 95308614.7
(22) Date of filing: 29.11.1995
(51) Int. Cl.: B41J 2/16

(54) **Bonding process for ink jet silicon chips**
Verbundverfahren für silizium Chips für den Tintenstrahldruck
Procédé de liaison pour puces au silicium pour jet d'encre

(30) Priority: 01.12.1994 US 347634
(43) Date of publication of application: 05.06.1996
(73) Proprietor: LEXMARK INTERNATIONAL, INC., Greenwich, Connecticut 06836 (US)
(72) Inventor: Christiansen, Robert Arnold, Salvisa, Kentucky 40372 (US); Eisele, Peter Jon, Lexington, Kentucky 40505 (US); Jackson, Tonya Harris, Nicholasville, Kentucky 40356 (US); Williams, Gary Raymond, Lexington, Kentucky 40517 (US)
(74) Representative: Skailes, Humphrey John

(56) References cited:
- US-A- 4 326 238
- US-A- 4 783 428
- US-A- 5 013 383
- US-A- 5 030 308

## Description

### FIELD OF THE INVENTION

The present invention is concerned with a process for bonding a silicon chip to the pen body of an ink jet printer.

### BACKGROUND OF THE INVENTION

Modern ink jet printing has placed many unprecedented demands upon materials and processes for assembling them. The present invention is concerned with a solution for one such demand, namely a process for bonding the silicon chip to the pen body of the ink jet printer.

The bond between the ink jet silicon chip and the pen body of the ink jet printer is subject to very severe attack, especially because in usage the temperature is very high and the bond is exposed to aqueous-base liquid inks commonly containing organic cosolvents and also having very high (alkaline) pH. Not only does the bond have to serve to attach the chip to the pen body, but it also has to form a leak resistant bond around the chip to prevent ink transfer to the user.

The bonding material also must be such that it does not change the properties of the ink used in the system, and in modern color printers three different inks are commonly used. Additionally, the cure temperature of the adhesive material must be below the glass transition temperature of the plastic which forms the pen body. To build a multicolor ink jet pen, the vias in the chip must be separated, generally by an adhesive, which serves as a barrier or sealant around each via to prevent ink mixing. Furthermore, the adhesive must serve as a gasket around the chip to prevent ink mixing. Furthermore, the adhesive must serve as a gasket around the chip to prevent inks from leaking to outside the body. Increasingly closer via spacing to provide ever-higher dots-per-inch (dpi) print resolution puts extreme demands on an adhesive to make a reliable bond in a very harsh environment.

A method for improving adhesion at the adhesive to silicon interface is necessary to prevent two failure possibilities. If an adhesive failure occurs at that interface, then the primary colors will flow freely, thereby resulting in ink mixing. Secondly, if the adhesive to chip interface fails at the perimeter, the ink will leak, and ink can be transferred to the user through routine handling. Both types of failures would be considered reliability failures.

### DISCLOSURE OF THE INVENTION

The present invention, which is defined in the independent claims, solves the problems mentioned above. According to this invention, the silicon chip is first covered with a thin coating of a silane coupling agent. This coating is applied on the side of the chip that does not contain the electronic circuitry. The coating of the silane coupling agent is in turn coated with a thin (about 0.5 to about 5.0 µm (microns)) layer of an epoxy resin, which is then cured at a temperature of about 175°C.

In a further mode of carrying out the present invention, the above steps are carried out on a multi-chip silicon wafer, which can then be subjected to subsequent manufacturing operations. Hundreds of chips can be treated on a single silicon wafer.

In the final step of the process of the present invention, the chip is attached to the pen body using an epoxy which cures at a temperature of 100°C or less.

### DESCRIPTION OF THE DRAWINGS

Understanding of the invention will be facilitated by reference to the accompanying drawings.
Figure 1 is a cross-sectional view, not to scale, of a coated silicon wafer.
Figure 2 is a cross-sectional view, not to scale, of an ink jet print head chip and pen portion.

In Figure 1, 1 is a silicon wafer; 2 is the circuitry on one side of the wafer; 3 is a layer of adhesion promoter; and 4 is a layer of epoxy resin.

In Figure 2, 1 is the pen body of the ink jet printer nozzle; 2 is the ink jet silicon chip; 3 is an acrylate based polymer thick film; 4 is the nozzle plate; 5 is a layer of rapid/low temperature cure epoxy adhesive; 6 is two thin layers, one of adhesion promoter and one of an epoxy resin; and 7 is the ink via.

### BEST MODE EXAMPLE

A preferred silane coupling agent is Dow Corning Z6032, a vinylbenzylamine functional silane. The commercial material is prehydrolyzed by adding 5% water by weight to the silane solution. It is then diluted to a 1% functional silane solution using ethanol. This solution is spread on the non-circuitry bearing side of the stationary silicon wafer and allowed to sit for 20-30 seconds. The wafer is then spun for 45 seconds at 2,000 RPM to remove the excess and dry the wafer surface.

A preferred high temperature cure epoxy is a tertiary amine cured compound such as Ablebond 968, from the Ablestik Co. This material is used without filler. It is first diluted with gamma butyrolactone in a 1 to 1 ratio. Approximately 2 mL of this solution is deposited in the center of the wafer after the silane has been deposited. The wafer is spun at 2,500 RPM for 45 seconds. This results in a uniform film of epoxy approximately 0.8 µm (microns) thick on the wafer. The wafer is then baked for 2 hours at 175°C to cure the epoxy.

Finally, the wafer is cut into individual chips, which are attached to the pen body by means of a polybenzimidazole low temperature curing epoxy, such as Emerson-Cuming LA3032-78, an epoxy which is cured at about 100°C.

For inkjet pen products, as they are consumable (often disposable) products, the manufacturing processes must incorporate low cost material that can be manufactured at high throughputs. Pen bodies are most commonly injection molded thermoplastic materials such as modified polyphenylene oxide (PPO). The elevated temperature resistance of such material sets a maximum cure temperature allowable for subsequent processes, such as attachment of the inkjet chip and nozzle assembly to the body.

Materials are available that cure in the 100°C or less range, and in short times, and that are resistant to ink formulations in bulk exposure. However, premature adhesion failures at the silicon to diebond adhesive interface are commonly observed. By applying the silane/ultrathin epoxy layer at an early stage of manufacture, (at the wafer level) hundreds of chips are coated and protected simultaneously. At this stage high purity, highly stoichiometric epoxies can be thoroughly cross-linked at the higher temperature (at least 175°C resulting in a much better attachment to the silane/silicon die). A method of enhancement of product life is then achieved while maintaining throughput economically.

The process of the present invention is characterized by the use of two different epoxy resins, the first of which cures at a temperature above the heat distortion temperature of the plastic pen body, and the second of which cures at a temperature below the heat distortion temperature of the plastic pen body. When attached to the pen body, the chips have an ink via extending into the chips bounded by the coupling agent, the first epoxy resin and the second epoxy resin.

Other features of this invention are the following: Insensitivity to manufacturing line interruption/processes (as a silane alone would be), and the ultrathin usage provides minimal thermal barrier addition to heat removal from the die.

## Claims

1. A process for bonding an ink jet silicon chip to the plastic pen body of an ink jet printer, said process comprising the steps of:
1) applying to the non-circuitry containing side of said chip a thin coating of a silane coupling agent;
2) applying on top of said coupling agent a thin coating of a first epoxy resin;
3) curing said first epoxy resin at a temperature above the heat distortion temperature of the plastic pen body;
4) attaching the coated chip to the plastic pen body by means of a second epoxy resin which is cured at a temperature below the heat distortion temperature of the plastic pen body

2. A process for bonding an ink jet silicon chip to the pen body of an ink jet printer, said process comprising the steps:
1) applying to the non-circuitry containing side of said chip a thin coating of a silane coupling agent;
2) applying on top of said coupling agent a thin coating of a first epoxy resin;
3) curing said first epoxy resin at a temperature of about 175°C; and
4) attaching the coated chip to the pen body by means of a second epoxy resin which is cured at a temperature of 100°C or less.

3. A process as claimed in claim 1 wherein the thin coating of the silane coupling agent and the thin coating of the first epoxy resin are each applied by a spinning process.

4. A process as claimed in claim 1 wherein the application of the thin coating of a silane coupling agent and the application of the thin coating of the first epoxy resin are carried out on a multi-chip silicon wafer.

5. A process as claimed in claim 1 wherein the thin coating of the first epoxy resin is about 0.5 to about 5.0 µm (microns) thick.

6. A process as claimed in claim 1 wherein the silane coupling agent is a vinylbenzylamine functional silane.

7. A process as claimed in any preceding claim wherein said chip, when attached to the pen body, has an ink via extending into said chip bounded by said coupling agent, said first epoxy resin and said second epoxy resin.

8. A process for bonding ink jet silicon chips to the pen body of an ink jet printer, said process comprising the steps:
1) spin coating the non-circuitry containing side of a multi-chip silicon wafer with a thin coating of a vinylbenzylamine functional silane;
2) spin coating said thin coating with a coating about 0.8 µm (microns) thick of a first epoxy resin;
3) curing said first epoxy resin at a temperature of about 175°C;
4) separating said multi-chip silicon wafer into individual chips; and
5) attaching said individual chips to the pen body by means of a second epoxy resin which is cured at a temperature of 100°C or less.

9. A process as claimed in claim 8 wherein the chips, when attached to the pen body, have an ink via extending into said chips bounded by said coupling agent, said first epoxy resin and said second epoxy resin.

## Patentansprüche

1. Verfahren zum Verbinden eines Tintenstrahl-Siliciumchips mit dem Kunststoffstiftkörper eines Tintenstrahldruckers, wobei das Verfahren die Schritte umfaßt:
1) Auftragen eines dünnen Überzugs eines Silan-Kupplungsmittels auf die Seite des Chips, die keine Schaltungsanordnung enthält;
2) Auftragen eines dünnen Überzugs eines ersten Epoxidharzes über dem Kupplungsmittel;
3) Härten des ersten Epoxidharzes bei einer Temperatur über der Formbeständigkeitstemperatur des Kunststoffstiftkörpers;
4) Anbringen des beschichteten Chips an dem Kunststoffstiftkörper mittels eines zweiten Epoxidharzes, das bei einer Temperatur unter der Formbeständigkeitstemperatur des Kunststoffstiftkörpers gehärtet wird.

2. Verfahren zum Verbinden eines Tintenstrahl-Siliciumchips mit dem Stiftkörper eines Tintenstrahldruckers, wobei das Verfahren die Schritte umfaßt:
1) Auftragen eines dünnen Überzugs eines Silan-Kupplungsmittels auf die Seite des Chips, die keine Schaltungsanordnung enthält;
2) Auftragen eines dünnen Überzugs eines ersten Epoxidharzes über dem Kupplungsmittel;
3) Härten des ersten Epoxidharzes bei einer Temperatur von etwa 175°C; und
4) Anbringen des beschichteten Chips an dem Stiftkörper mittels eines zweiten Epoxidharzes, das bei einer Temperatur von 100°C oder weniger gehärtet wird.

3. Verfahren nach Anspruch 1, bei dem der dünne Überzug des Silan-Kupplungsmittels und der dünne Überzug des ersten Epoxidharzes jeweils durch ein Schleuderverfahren aufgebracht werden.

4. Verfahren nach Anspruch 1, bei dem der Auftrag des dünnen Überzugs eines Silan-Kupplungsmittels und der Auftrag des dünnen Überzugs des ersten Epoxidharzes auf einem Mehrchip-Siliciumwafer ausgeführt werden.

5. Verfahren nach Anspruch 1, bei dem der dünne Überzug des ersten Epoxidharzes etwa 0,5 bis etwa 5,0 µm (Mikron) dick ist.

6. Verfahren nach Anspruch 1, bei dem das Silan-Kupplungsmittel ein Vinylbenzylamin-funktionelles Silan ist.

7. Verfahren nach einem vorangehenden Anspruch, bei dem der Chip, wenn er an dem Stiftkörper angebracht ist, einen Tintenweg aufweist, der sich, begrenzt vom Kupplungsmittel, dem ersten Epoxidharz und dem zweiten Epoxidharz, in den Chip erstreckt.

8. Verfahren zum Verbinden von Tintenstrahl-Siliciumchips mit dem Stiftkörper eines Tintenstrahldruckers, wobei das Verfahren die Schritte umfaßt:
1) Schleuderbeschichten der Seite eines Mehrchip-Siliciumwafers, die keine Schaltungsanordnung enthält, mit einem dünnen Überzug eines Vinylbenzylamin-funktionellen Silans;
2) Schleuderbeschichten des dünnen Überzugs mit einem etwa 0,8 µm (Mikron) dicken Überzug eines ersten Epoxidharzes;
3) Härten des ersten Epoxidharzes bei einer Temperatur von etwa 175°C;
4) Aufteilen des Mehrchip-Siliciumwafers in einzelne Chips; und
5) Anbringen der einzelnen Chips an dem Stiftkörper mittels eines zweiten Epoxidharzes, das bei einer Temperatur von 100°C oder weniger gehärtet wird.

9. Verfahren nach Anspruch 8, bei dem die Chips, wenn sie an dem Stiftkörper angebracht sind, einen Tintenweg aufweisen, der sich, begrenzt vom Kupplungsmittel, dem ersten Epoxidharz und dem zweiten Epoxidharz, in die Chips erstreckt.

## Revendications

1. Procédé de liaison d'une puce au silicium pour jet d'encre à la tête d'impression plastique d'une imprimante à jet d'encre, ledit procédé comprenant les étapes :
1) d'application sur le côté ne contenant pas de circuits de ladite puce d'un mince revêtement d'un agent de couplage de type silane ;
2) d'application sur ledit agent de couplage d'un mince revêtement d'une première résine époxy;
3) de durcissement de ladite première résine époxy à une température supérieure à la température de déformation à la chaleur de la tête d'impression plastique;
4) de fixation de la puce revêtue à la tête d'impression plastique au moyen d'une seconde résine époxy qui est durcie à une température inférieure à la température de déformation à la chaleur de la tête d'impression plastique.

2. Procédé de liaison d'une puce au silicium pour jet d'encre à la tête d'impression plastique d'une imprimante à jet d'encre, ledit procédé comprenant les étapes :
1) d'application sur le côté ne contenant pas de circuits de ladite puce d'un mince revêtement d'un agent de couplage de type silane ;
2) d'application sur ledit agent de couplage d'un mince revêtement d'une première résine époxy;
3) de durcissement de ladite première résine époxy à une température d'environ 175°C; et
4) de fixation de la puce revêtue à la tête d'impression plastique au moyen d'une seconde résine époxy qui est durcie à une température de 100°C ou moins.

3. Procédé suivant la revendication 1, dans lequel le mince revêtement de l'agent de couplage de type silane et le mince revêtement de la première résine époxy sont appliqués chacun par un traitement centrifuge.

4. Procédé suivant la revendication 1, dans lequel l'application du mince revêtement d'un agent de couplage de type silane et l'application du mince revêtement de la première résine époxy sont réalisées sur une plaquette de silicium multipuce.

5. Procédé suivant la revendication 1, dans lequel le mince revêtement de la première résine époxy a une épaisseur d'environ 0,5 à environ 5,0 µm.

6. Procédé suivant la revendication 1, dans lequel l'agent de couplage de type silane est un silane fonctionnel vinylbenzylamine.

7. Procédé suivant l'une quelconque des revendications précédentes, dans lequel ladite puce, lors qu'elle est attachée à la tête d'impression, comprend un passage pour l'encre qui se prolonge dans ladite puce liée par ledit agent de couplage, ladite première résine époxy et ladite seconde résine époxy.

8. Procédé de liaison pour puces au silicium pour jet d'encre à la tête d'impression plastique d'une imprimante à jet d'encre, ledit procédé comprenant les étapes :
1) d'application centrifuge sur le côté ne contenant pas de circuits d'une plaquette de silicium multipuce d'un mince revêtement d'un silane fonctionnel vinylbenzylamine ;
2) d'application centrifuge sur ledit mince revêtement d'un revêtement d'environ 0,8 µm d'épaisseur d'une première résine époxy;
3) de durcissement de ladite première résine époxy à une température d'environ 175°C;
4) de séparation de ladite plaquette de silicium multipuce en puces individuelles; et
5) de fixation desdites puces individuelles à la tête d'impression au moyen d'une seconde résine époxy qui est durcie à une température de 100°C ou moins.

9. Procédé suivant la revendication 8, dans lequel les puces, lorsqu'elles sont attachées à la tête d'impression, comprennent un passage pour l'encre qui se prolonge dans lesdites puces liées par ledit agent de couplage, ladite première résine époxy et ladite seconde résine époxy.
